

Aug. 10, 1965

A. DAMMER ET AL

3,199,976

MANUFACTURE OF STEEL

Filed June 17, 1964



Inventors:

AUGUST DAMMER, WILHELM BREVING

By Burgess, Dinklage & Sprung  
ATTORNEYS

1

3,199,976

## MANUFACTURE OF STEEL

August Dammer, Viersen, and Wilhelm Breuig, Bochum, Germany, assignors to Rheinstahl Hüttenwerke AG., Essen, Germany, a German corporation

Filed June 17, 1964, Ser. No. 375,746

Claims priority, application Germany, Dec. 1, 1960, R 29,203; June 26, 1963, R 35,512  
12 Claims. (Cl. 75—59)

This application is a continuation-in-part of our pending application, Serial No. 157,300 filed November 28, 1961, now abandoned, for Manufacture of Steel.

This invention relates to new and useful improvements in the manufacture of steel. The invention more particularly relates to a process for reducing the hydrogen content of steel melts without the necessity of vacuum.

Too high a content of hydrogen in steel may adversely affect the characteristics of steel, as for example the tendency to flake.

Thus, for example, it is generally considered desirable to reduce the hydrogen content of steel which is to be worked by rolling to below 3.0 cu. cm./100 grams and to below 2.0 cu. cm./100 grams for steel which is to be worked by forging.

In the past, in order to obtain these low hydrogen contents, it was necessary to degas the steel melt under a high vacuum below 1 torr and as low as .05 to .3 torr. The vacuum degassing could be effected by passing a stream of molten steel into a vacuum chamber by maintaining a bath of the molten steel in a chamber maintained under low vacuum and preferably while passing a scavenging gas into or through the steel or the like. Vacuum degasification requires the use of special, expensive vacuum equipment and pumps and often the steel melt treated must be free of a slag covering layer.

One object of this invention is the reduction of the hydrogen content of steel melts without the requirement of the application of a vacuum.

A further object of this invention is a simplified process for removing hydrogen from steel which may be combined with the blowing of iron melts to steel.

These and still further objects will become apparent from the following description read in conjunction with the drawing which diagrammatically shows an arrangement for effecting the process in accordance with the invention.

In accordance with the invention, we have discovered that the hydrogen content of steel melts may be reduced to a value previously only obtainable with a high vacuum degasification by maintaining a bath of the molten steel with slag covering the surface thereof and blowing a stream of oxygen and .5 to 7% by volume and preferably 1 to 5% by volume, based on said oxygen, of a lower chlorinated or fluorochlorinated alkane against the slag with a velocity sufficient to cause intermixing of the slag and at least the upper portion of the bath.

The term "steel" as used herein includes any of the known or conventional steels, such as alloyed, unalloyed steels, and includes iron melts from which steel is ultimately produced, as for example, molten pig iron.

The slag which covers the surface of the molten steel bath treated in accordance with the invention may be any known or conventional slag and is generally the conven-

2

tional slag used in the production of the particular steel in question.

While the content of the slag is not critical and does not affect the treatment in accordance with the invention, the slags generally have the following components:

|                  | Percent b.w. |
|------------------|--------------|
| CaO              | 30-65        |
| MnO              | 5-25         |
| SiO <sub>2</sub> | 10-30        |

10 Remainder iron oxides, magnesia and, if any, fluxing means preferably CaF<sub>2</sub>.

Similarly the thickness of the slag layer is not critical and is generally that conventionally found in the production of steel, as for example, between 2 and 6 cm.

15 The chlorine-containing material which is blown against the slag with the oxygen may be a lower hydrocarbon having all of its hydrogen atoms substituted with chlorine or chlorine and fluorine. As lower hydrocarbons, any

20 completely chlorinated or completely fluorochlorinated hydrocarbon having 4 or less carbon atoms may be used but preferably the hydrocarbon should not have more than 2 carbon atoms. Carbon tetrachloride has proven most preferably but very good results are obtained with

25 hexachloroethane or difluorodichloroethane or the like. It is also possible to use mixtures of these lower chlorinated or fluorochlorinated ethanes.

20 The steel melt with the slag covering is maintained in any suitable container used in the steel industry, as for example a furnace crucible or ladle, and the oxygen and chlorine-containing material is blown against the surface through any convenient nozzle or lance or nozzles or lances.

30 It is not necessary to change the lances and nozzles suitable for the processes in which oxygen is blown on or into a steel bath, as known in open hearth or electric furnaces or LD-crucibles. This is true for the distance between nozzles or lances from the surface of slag surface as known, the distances vary between 300 and 2000 millimeters.

35 The blowing should be effected with sufficient velocity to cause intermixing of the slag and at least the upper portion of the melt. This velocity will vary in individual cases depending on the conditions, etc. In general, however, a velocity of at least 200 meters/second, preferably 700-800 meters/second, have proven suitable.

40 The chlorine-containing material and oxygen pass through the same nozzles with the chlorine material being fed into the oxygen stream, as for example by use of a conventional dosing pump.

45 It is preferred to blow all oxygen together with the chlorine containing material but it is also possible to blow only a portion of the oxygen together with said additional material and to blow the remaining portion of oxygen through an additional lance or nozzle or additional lances or nozzles.

50 The amounts of oxygen may vary over wide limits, as for example between 33 and 100 normal cu. meters per metric ton of steel.

55 The total amount of the chlorine containing material used is also dependent upon the conditions and the degree of reduction of the hydrogen content. In general however, amounts of .3 to 1.5 normal cu. meters may be required per metric ton of steel treated.

The treatment in accordance with the invention may be effected at any stage in the production of the steel after the melt has been formed and may be used in conjunction with any of the known or conventional methods of producing steel in any of the known or conventional furnaces.

Most preferably, however, the treatment is combined with the production of steel involving an oxygen blowing of the melt as for example in the LD process utilizing for example an LD crucible. In accordance with the invention, the blowing of the oxygen onto the surface of the pig iron bath to convert it to steel may be combined with the treatment in accordance with the invention by including the chlorine-containing material into the oxygen used for the blowing.

In other steelmaking processes or open hearth and electric furnace process the treatment is effected in a similar manner.

The treatment in accordance with the invention may be started at a point in the steel production where the slag layer is replaced by different slag layer. If the treatment has been started before the slag was replaced by a new slag, it has been found preferable to subject the steel after replacement of the slag layer with a blowing with oxygen and the chlorine-containing material in accordance with the invention.

4  
a hot blast cupola furnace and which had the following approximate analysis:

|    |       |       |
|----|-------|-------|
| C  | ----- | 4.0   |
| Si | ----- | 0.10  |
| Mn | ----- | 0.45  |
| P  | ----- | 0.050 |
| S  | ----- | 0.020 |

To each of the charges 900 kg. lime and 300 kg. fluor-spar were added before blowing. Each of the charges was blown with oxygen passed through the lance 2, which was maintained at a distance of 800 mm. from the surface of the slag. The gas pressure in the lance was maintained at between 4 and 6 atmospheres, and the nozzle velocity of the gas emitted from the lance was between 700 and 800 meters per second.

As a Laval-Nozzle was used the velocity of the gas striking the slag was substantially the same. The nozzle outlet diameter of the lance was 30 millimeters, and 1650 normal cu. meters oxygen were passed through the lance.

Carbon tetrachloride was fed into the oxygen lance 2 by means of the dosing pump 3 at a constant rate.

Table I below shows the total carbon tetrachloride blown into each of the charges, the blowing time for each of the charges, the analysis of steel melt produced and the hydrogen content as analyzes by two individually taken samples from each charge:

Table I

| Charge No. | Total amount of CCl <sub>4</sub> blown, in liters | Blowing time, minutes | Final analyses of the steel |     |     |      |      |     |       |      | H <sub>2</sub> content, p.p.m. |          |
|------------|---------------------------------------------------|-----------------------|-----------------------------|-----|-----|------|------|-----|-------|------|--------------------------------|----------|
|            |                                                   |                       | C                           | Si  | Mn  | P    | S    | Cr  | Cu    | Al   | Sample 1                       | Sample 2 |
| 1          | 78 (18 Nm <sup>3</sup> )                          | 27                    | .09                         | .22 | .36 | .014 | .026 | .20 | .21   | .007 | 1.44                           | 1.44     |
| 2          | 80 (18.5 Nm <sup>3</sup> )                        | 25                    | .08                         | .25 | .37 | .007 | .024 | .12 | .13   | .002 | .88                            | .88      |
| 3          | 82 (19 Nm <sup>3</sup> )                          | 25                    | .10                         | .19 | .35 | .012 | .024 | .18 | ----- | .005 | .96                            | 1.04     |

Furthermore, if after the treatment the melt is to be maintained so that it would normally be in contact with the ambient air as would occur, for example, by a delay in tapping or pouring, it has been found preferable to maintain the steel free from contact with this ambient air by flowing with an inert gas with or without chlorine-containing material. This is done to prevent a rise in the hydrogen content of the melt which could occur through the absorption of hydrogen from the moisture in the ambient air. The expression "inert gas" does not mean only argon, helium etc., but means all gases which do not affect the bath.

Thus, for example, waste gas, as for example, blast furnace or hot cupola gas may be used, being blown on the surface of the melt at a sufficient rate to prevent contact with the air. It has been found that even a small hydrogen content of, for example about 1-2% hydrogen in such gas is not detrimental.

The following examples are given by way of illustration and not limitation:

## EXAMPLE 1

An arrangement consisting of an LD-crucible and a lance as shown in FIG. 1 is utilized for treatment. In the drawing the LD-crucible is designated with 1, the lance capable of being raised and lowered is designated with 2. The dosing pump 3 has to pump the fluid CCl<sub>4</sub> from a container 4 by means of a pressure conduit 5 at 6 into the lance 2 and thereby into a stream of oxygen. 7 is the tapping hole.

The LD-crucible 1 which had a capacity of 35 metric tons was charged with 3 separate charges of pig iron which had been produced from scrap iron and coke in

45  
50  
55  
The hydrogen content analysis was determined by means of a hot aging determination at 600° C. (see: "Mitteilungen des Kaiser Wilhelm Institut für Eisenforschung" Vol. XIX (1937). Lfg. 8, page 105-112 and "Iron and Coal," 15. 8. 1960, page 301-304).

In comparison thereto identical melts were blown under the substantially identical conditions without the CCl<sub>4</sub>, however, the hydrogen content was above 4.0 p.p.m. and the steel melt produced had the following analysis:

|    |       |      |
|----|-------|------|
| C  | ----- | .13  |
| Si | ----- | .27  |
| Mn | ----- | .33  |
| P  | ----- | .020 |
| S  | ----- | .015 |
| Cr | ----- | .05  |
| Al | ----- | .005 |

## EXAMPLE 2

Example 1 was repeated except that the CCl<sub>4</sub> was replaced by the following chlorine-containing materials:

- Hexachloroethane
- Dichlorodifluoroethane
- Decachlorobutane
- Mixtures of the above.

In each case the hydrogen content of the melt is reduced to below 1.6 p.p.m.

## EXAMPLE 3

Example 1 was further repeated except that the 50% of the slag was withdrawn after a blowing period of 14 minutes together with 44 liters (10.3 normal cubic meters) CCl<sub>4</sub>. After adding of 120 kg. lime and 120 kg. fluor-spar blowing was continued for 17 minutes with the result that hydrogen content was 1.8 p.p.m.

In a steel containing: .12 C, .24 Si, .38 Mn, .014 P, .024 S, .19 Cr, .20 Cu, .008 Al, all percents by weight, in the final analysis.

While the invention has been described in detail with reference to certain specific embodiments, various changes and modifications which fall within the spirit of the invention and scope of the appended claims will become apparent to the skilled artisan. The invention is therefore only intended to be limited by the appended claims or their equivalents wherein we have endeavored to claim all inherent novelty.

We claim:

1. Process for reducing the hydrogen content of steel melts, which comprises maintaining a bath of molten steel with slag covering the surface thereof and blowing a stream of oxygen and .5 to 7% by volume, based on said oxygen, of a member selected from the group consisting of lower completely chlorinated alkanes, lower completely fluorochlorinated alkanes, and mixtures thereof, against the slag with a velocity sufficient to cause intermixing of the slag and the upper portion of the bath for a period of time sufficient to substantially reduce the hydrogen content of the melt.

2. Process according to claim 1 in which said group member is blown in said stream of oxygen.

3. Process according to claim 1 in which said group member is utilized in amount of about 1 to 5% by volume, based on said oxygen.

4. Process according to claim 1 in which said group member is  $\text{CCl}_4$ .

5. Process according to claim 1 in which said group member is utilized in amount of .3 to 1.5 normal cu. meters per metric ton of steel treated.

6. Process according to claim 1 in which the bath of molten steel is maintained at normal pressure.

7. Process according to claim 1 which includes protecting the melt with an inert gas from prolonged contact with moisture-containing ambient atmosphere after said treatment.

5 8. In a process for blowing iron to steel in which a stream of oxygen is blown against a bath of slag covered molten iron, the improvement for producing steel with a lowered hydrogen content which comprises effecting the blowing with a stream of oxygen additionally containing .5 to 7% by volume of a member selected from the group consisting of lower completely chlorinated alkanes, lower completely fluorochlorinated alkanes, and mixtures thereof.

15 9. Improvement according to claim 8 in which said group member is present in amount of about 1 to 5% by volume.

10 10. Improvement according to claim 8 in which said group member is  $\text{CCl}_4$ .

20 11. Process according to claim 1 which includes removing said slag from said bath of molten steel, covering the surface of said bath of molten steel with a different slag and continuing said blowing against the new slag.

25 12. Process according to claim 1, in which said oxygen is blown in at least two separate streams, at least one of said streams containing said group member.

#### References Cited by the Examiner

#### UNITED STATES PATENTS

|    |           |       |                 |        |
|----|-----------|-------|-----------------|--------|
| 30 | 2,068,785 | 1/37  | Bain            | 75-12  |
|    | 2,770,860 | 11/56 | Webbere         | 22-214 |
|    | 3,046,107 | 7/62  | Nelson et al.   | 75-60  |
|    | 3,060,015 | 10/62 | Spolders et al. | 75-60  |

35 BENJAMIN HENKIN, Primary Examiner.